

## UNITED STATES PATENT OFFICE

WILLIAM D. TREADWELL, OF ZURICH, SWITZERLAND, ASSIGNOR TO ALUMINUM INDUSTRIE AKTIENGESELLSCHAFT, OF NEUHAUSEN, SWITZERLAND, A JOINT-STOCK COMPANY OF SWITZERLAND

## ELECTROLYTIC REFINING OF METALLIC ALUMINUM

No Drawing. Application filed November 30, 1929, Serial No. 410,878, and in Germany November 30, 1928.

This invention relates to the electrolytic refining of metallic aluminum, and consists in a novel process for producing highly pure metallic aluminum from less pure metal. 5  
 5 The invention is directed particularly to the extraction of refined aluminum from pig or ingot aluminum, aluminum alloys and the like. It constitutes an improvement more particularly in that refining processes where-  
 10 in the electrodes, used in a solid form, are im- mersed in a molten electrolyte, for example containing halogen salts, which electrolyte has a melting point lower than that of either electrode and is maintained in a molten con-  
 15 dition below the melting point of either elec- trode. Such a process has been described in and made the subject of patent of Weber and Hauser, No. 1,709,759, granted April 16, 1929, and of application of Weber and Zeerleder,  
 20 Serial No. 195,861, filed June 1, 1927, which may be referred to for details and features not herein fully described.

The general object of the present invention is to render more efficient the refining process, 25 and to enlarge the rate of output or produc-  
 25 tion. A particular object is to provide a treatment or step for purifying the electrodes upon their removal from the electrolytic bath by freeing them from the salts of the bath  
 30 which tend to adhere thereto. A further ob- ject is to increase the practical economy of the process by recovering and rendering available for further use substantially the entire quantity of electrolyte material so ad-  
 35hering to and removed with the electrodes, and without impairment or change in the chemical composition thereof. Other objects and advantages of the invention will be explained in the hereinafter following descrip-  
 40 tion of an illustrative embodiment thereof or will be understood to those conversant with the subject. To the attainment of such ob- jects and advantages the present invention consists in the novel electrolytic refining  
 45 process and the novel steps, operations and agents herein described.

The present improved process can best be explained by first pointing out certain con- ditions which pertain to the process as al-  
 50 ready known and the consideration in-

volved in further perfecting the same. In practicing the described refining process I have observed that on lifting the electrodes out of the electrolytic bath they are in an undesirable condition due to carrying or being covered with substantial quantities of the salts constituting the electrolytic bath. The amount of such electrolyte material is substantially larger in the case of the anodes from which the aluminum has been exhaust- 55 ed than in the case of cathodes. This is due to the fact that the electrolyte not only ad-heres to the surface of the electrodes, but tends also to penetrate into the narrow canals and pores left in the anode by the extraction of aluminum, which latter may in some cases be replaced by an approximately equal volume of salts of the electrolyte. 60

In the case of the anode, and taking the specific gravity of the electrolyte as 1.7 then 70 the exhausted anode will contain for every kilogram of refined aluminum removed from it 630 grams of electrolyte material, in ad- dition to the amount thereof which adheres to the surface. We have found that the total amount of the electrolyte which cannot read- 75 ily be separated by mechanical means from the anode will amount in general to 700 to 800 grams for every kilogram of refined alum- 80 inum, when the specific gravity of the electro- lyte is 1.7.

This substantial loss of electrolyte mate- rial impaired the economy and efficiency of the process, and constituted a practical prob- 85 lem in the perfecting of the process. Addi- tionally, the subsequent working and utili- zation of the electrodes is rendered much more difficult by reason of the presence of the elec- trolyte adhering to them, especially because the readily volatile aluminum chloride com- 90 pels special precautions to be taken in the melting of the electrodes. Furthermore the strongly hydroscopic character of the elec- trolyte renders it impracticable to store the anodes in uncleaned condition after removal 95 from the bath, since the electrolyte material deliquesces under the influence of atmos- pheric moisture and tends to produce crum- bling of the electrodes.

It is entirely insufficient and impractical 100

to wash the removed electrodes with water, for several reasons. Thus, the electrolyte can not be easily recovered from the aqueous solution owing to the decomposition of the aluminum salts. Further, such an aqueous solution of the electrolyte salts, being decidedly acid, would tend to dissolve a quite appreciable amount of aluminum from the electrodes and thus bring about losses impairing the economies of the process.

The main purpose therefore of the present invention is to permit the absorbed and adhering electrolyte material to be readily and completely extracted and separated from the electrodes in a simple and economical manner, leaving the electrodes in suitable condition, and conserving the salts for repeated use.

The present improved process is based upon the determination that the salt mixture employed as an electrolyte in the previously described process of refining metallic aluminum is readily soluble in anhydrous sulfur dioxide. This solvent is further advantageous in that no decomposition of the salts forming the electrolyte take place, and moreover the entire amount of such salts are quite readily recovered by the mere distilling off of the solvent. This capability of anhydrous sulfur dioxide to dissolve in substantial quantities such a salt mixture was not to be expected, since the respective salts which enter the composition of the electrolyte, if treated separately, are dissolved only in very small amounts, insufficient for practical purposes. Thus for example, 100 parts of anhydrous sulfur dioxide will dissolve at most five parts of the chlorides of aluminum or sodium or potassium respectively if brought individually into contact with the solvent. The same quantity of the solvent will however dissolve a far greater proportion, in some cases up to 170 parts, of an electrolyte such as that described in the prior application of Weber and Zeerleder, containing these same chlorides of aluminum, sodium and potassium, with more than one molecule of aluminum chloride present for each molecule of the alkali chlorides.

The treatment of the electrodes with the described solvent consisting of or containing anhydrous sulfur dioxide may be carried out by dipping or immersion in any sort of extraction apparatus or vessel commonly used in the chemical industries, provided that they are adapted to use with the said solvent. I prefer the use of apparatuses which permit a continuous extraction of the salts as for instance known apparatuses constructed in accordance with the Soxhlet principle. However, the treatment may be otherwise. It is even feasible to bring the electrodes into contact with gaseous sulfur dioxide provided that the latter is caused to condense upon the

electrodes, since in the gaseous state it of course can not act as a solvent.

The present invention may be summed up specifically as relating to that process of producing refined metallic aluminum comprising removing aluminum electrolytically from a solid metallic anode containing impure metallic aluminum on to a solid cathode through a molten electrolytic bath capable of acting selectively to dissolve aluminum from the anode, which bath contains aluminum halide, and the halides of one or more metals, such as the alkali metals or the alkali earth metals, the hydroxides of which have alkaline properties, and the improvement characterized in that the electrolyte material which is absorbed by or adheres to the electrodes, or either of them, after their removal from the electrolytic bath, is separated from them and recovered by treating the electrodes with a volatile solvent such as anhydrous sulfur dioxide, this solvent being afterwards distilled off from the resulting solution so as to leave the salt mixture available for further use as an electrolyte.

Within the principles of the above described improvement certain variations or equivalent steps may be employed. It is believed that, in the process of electrolytically refining aluminum which comprises the employment of solid electrodes in an electrolyte of molten salts, it is now with the present invention to perform the step of clearing or freeing one or both of the electrodes of salts adhering thereto upon their removal from the electrolyte by treatment with a suitable volatile solvent, thus not merely cleaning the electrodes but rendering the electrolyte material available for further use. While we have disclosed as a suitable volatile solvent anhydrous sulfur dioxide  $\text{SO}_2$ , various other volatile, and preferably anhydrous, solvents are available, among which may be mentioned  $\text{SOCl}_2$  and  $\text{SO}_2\text{Cl}_2$ , which however, although effective as solvents, are not so advantageous in a commercial sense on account of their higher cost and greater difficulty in handling.

There has thus been described a process for producing pure metallic aluminum from the less pure metal, together with special treatments or procedure for the improvement of the process and the product thereof, and a special agent or solvent for use therein, embodying the principles and attaining the objects of the present invention. Since various matters of process, ingredient and apparatus may be variously modified without departing from the principles of the invention, it is not intended to limit the invention to such matters except so far as set forth in the appended claims.

What is claimed is:

1. The process of producing refined metallic aluminum, comprising removing aluminum electrolytically from a solid metallic

anode containing impure metallic aluminum, on to a solid cathode, through a molten electrolytic bath capable of acting selectively to dissolve aluminum from the anode, which  
5 bath contains aluminum halide, and halides of one or more metals the hydroxides of which have alkaline properties, and characterized in that the electrolyte absorbed by or adhering to the electrodes after their removal from  
10 the electrolytic bath is separated from them and recovered by treating the electrodes with anhydrous sulfur dioxide, the anhydrous sulfur dioxide being afterwards distilled off from the resulting solution, leaving the salt  
15 mixture available for further use.

2. In the process of electrolytically refining aluminum comprising the employment of solid electrodes in a molten electrolyte comprising a mixture of halide salts, the step  
20 of clearing one or both electrodes of salts adhering thereto upon removal from the electrolyte by treatment with a volatile anhydrous solvent.

3. In the process of electrolytically refining aluminum comprising the employment of solid electrodes in a molten electrolyte comprising a mixture of aluminum halide and the halides of one or more metals the hydroxides of which have alkaline properties, the step of  
30 clearing one or both electrodes of salts adhering thereto upon removal from the electrolyte by treatment with a volatile solvent containing anhydrous sulfur dioxide.

4. In the process of electrolytically refining aluminum comprising the employment of solid electrodes in an electrolyte of molten salts, the step of clearing one or both electrodes of salts adhering thereto upon removal from the electrolyte by treatment with  
40 a solvent consisting of a volatile anhydrous agent.

5. In the process of electrolytically refining aluminum comprising the employment of solid electrodes in an electrolyte of molten salts, the step of clearing one or both electrodes of salts adhering thereto upon removal from the electrolyte by treatment with a solvent consisting of a volatile anhydrous sulfur compound.

50 In testimony whereof, this specification has been duly signed by:

WILLIAM D. TREADWELL.

**CERTIFICATE OF CORRECTION.**

**Patent No. 1,816,304.**

**Granted July 28, 1931, to**

**WILLIAM D. TREADWELL.**

**It is hereby certified that the name of the assignee in the above numbered patent was erroneously written and printed as "Aluminum Industrie Aktiengesellschaft, of Neuhausen, Switzerland, a joint-stock company of Switzerland", whereas said name should have been written and printed as Aluminium Industrie Aktiengesellschaft, of Neuhausen, Switzerland, a joint-stock company of Switzerland, as shown by the records of assignments in this office; and that the said Letters Patent should be read with this correction therein that the same may conform to the record of the case in the Patent Office.**

**Signed and sealed this 22nd day of September, A. D. 1931.**

**M. J. Moore,  
Acting Commissioner of Patents.**

**(Seal)**